

# UNITED STATES PATENT OFFICE.

OYSTEIN RAVNER AND VICTOR MORITZ GOLDSCHMIDT, OF CHRISTIANIA, NORWAY,  
ASSIGNORS TO DET NORSKE AKTIESELSKAB FOR ELEKTROKEMISK INDUSTRI, NORSK  
INDUSTRI-HYPOTEKBANK, OF CHRISTIANIA, NORWAY.

## PROCESS OF PRODUCING ALUMINIUM COMPOUNDS.

1,302,852.

Specification of Letters Patent.

Patented May 6, 1919.

No Drawing.

Application filed March 19, 1917. Serial No. 155,883.

To all whom it may concern:

Be it known that we, OYSTEIN RAVNER, a subject of the King of Norway, residing at Christiania, Norway, and VICTOR MORITZ GOLDSCHMIDT, a subject of the King of Norway, residing at Christiania, Norway, have invented certain new and useful Improvements in Processes of Producing Aluminium Compounds; and we do hereby declare the following to be a full, clear, and exact description of the invention, such as will enable others skilled in the art to which it appertains to make and use the same.

Our invention relates to the treatment of rock-forming minerals of the feldspar group for the purpose of producing aluminium compounds poor in or free from iron.

As known from the literature it has been suggested to decompose aluminium silicates by different means. Although some of the methods proposed have, for the most part been technically possible, they have been uneconomical.

It can be readily understood that the economic production of aluminium compounds from minerals requires that the minerals be rich in aluminium and be readily available at a comparatively low price.

The co-inventor Goldschmidt and his associates have discovered processes whereby minerals rich in plagioclases particularly of the labradorite-anorthosite series are available and can be utilized for this purpose, and this application deals with one of the said processes. The use of minerals of this class is particularly advantageous in that they contain large quantities of combined aluminium (25-36 per cent.  $Al_2O_3$ ) and but little iron, the iron being combined with other metals present in compounds which are not readily acted upon and consequently remaining so that what little iron is present is wholly or in large part in the residue. The minerals referred to as containing the iron are principally hypersthene, diallage, epidote and similar minerals.

Our invention contemplates the treatment of minerals of the class just described with acid gases, the minerals meanwhile being maintained at a high temperature. Chlorin or hydrochloric acid gas and the oxids of nitrogen have been found to be particularly well adapted for this purpose.

In using chlorin or hydrochloric acid gas, it is of advantage to supply a reducing agent such as carbon. The aforesaid minerals together with a small quantity of carbon are subjected to the requisite temperature, for instance, 600° to 1000° C., and simultaneously supplied with the chlorin or hydrochloric acid gas. The combined aluminium in the minerals is acted upon and aluminium chlorid formed. This sublimates and can be gathered in a reservoir.

When the oxids of nitrogen are employed they are introduced into the furnace along with steam, the minerals being maintained at such a temperature that the combined sodium and calcium present are transformed into nitrates while the aluminium remains as an oxid. The decomposition mass is then lixiviated to remove the aforesaid nitrates. The residue, containing aluminium oxid, silicic acid, and possibly some combined iron, is then treated with an acid, such as nitric acid or sulfuric acid, which affects only the aluminium oxid, and a solution formed from which aluminium hydroxid can be recovered in any well known manner as by precipitation with ammonium hydroxid. Obviously the ammonium salts remaining in the solution can be recovered by evaporation.

The foregoing detailed description has been given for clearness of understanding, and no undue limitation should be deduced therefrom, but the appended claims should be construed as broadly as permissible in view of the prior art.

What we claim as new and desire to secure by Letters Patent of the United States is:

1. The process of producing an aluminium compound from minerals rich in plagioclases of the labradorite-anorthosite series, which comprises subjecting the minerals to the combined action of heat and a decomposing agent in the form of a gas, whereby salts are formed and combined aluminium is liberated, and recovering the aluminium compound from the decomposition mass.

2. The process of producing aluminium chlorid from minerals rich in plagioclases of the labradorite-anorthosite series, which comprises subjecting the minerals to the action of chlorin in the presence of a reducing

agent at such a temperature that aluminium chlorid is formed while the combined iron remains for the most part in the residue.

3. The process of producing aluminium chlorid from minerals rich in plagioclases of the labradorite-anorthosite series, which comprises subjecting the minerals to the action of chlorin in the presence of a reducing agent at temperatures from about 600° to 1000° C whereby aluminium chlorid is formed while the combined iron remains for the most part in the residue, and recovering the aluminium chlorid.

4. The process of producing aluminium chlorid from minerals rich in plagioclases of the labradorite-anorthosite series, which

comprises subjecting the minerals to the action of chlorin in the presence of carbon at temperatures from about 600° to 1000° C. whereby aluminium chlorid is formed while the combined iron remains for the most part in the residue, and recovering the aluminium chlorid by sublimation and condensation.

In testimony that we claim the foregoing as our invention, we have signed our names in presence of two subscribing witnesses.

OYSTEIN RAVNER.

VICTOR MORITZ GOLDSCHMIDT.

Witnesses:

C. VORMAN,

KARL L. LEE.